

1,383,628.

T. B. MUNROE.

PLASTER BOARD OF FIBROUS MATERIAL.  
APPLICATION FILED SEPT. 30, 1919.

Patented Mar. 16, 1920.

Fig. 1.



Fig. 4.



Fig. 2.



Fig. 5.



Fig. 3.



Fig. 6.



Fig. 7.



Highly porous, loosely compacted mass of fibers of different lengths and varying diameters.

T. B. Munroe by  
D. W. Witherup

Attorney

# UNITED STATES PATENT OFFICE.

TREADWAY B. MUNROE, OF FOREST GLEN, MARYLAND, ASSIGNOR TO B. G. DAHLBERG,  
OF ST. PAUL, MINNESOTA.

## PLASTER-BOARD OF FIBROUS MATERIAL.

1,333,628.

Specification of Letters Patent. Patented Mar. 16, 1920.

Application filed September 30, 1919. Serial No. 327,540.

To all whom it may concern:

Be it known that I, TREADWAY B. MUNROE, a citizen of the United States, residing at Forest Glen, in the county of Montgomery and State of Maryland, have invented certain new and useful Improvements in Plaster-Board of Fibrous Material; and I do hereby declare the following to be a full, clear, and exact description of the invention, such as will enable others skilled in the art to which it appertains to make and use the same.

This invention relates to a plaster board of fibrous material and has for its object to provide an article of this kind which will be less costly to manufacture and more efficient in use than those heretofore proposed.

With these and other objects in view the invention consists in the novel details of construction more fully hereinafter disclosed and particularly pointed out in the claims.

Referring to the accompanying drawings forming a part of this specification in which like numerals refer to like parts in all the views:

Figure 1 is a diagrammatic partly sectional view of a plaster board made in accordance with this invention;

Fig. 2 is a cross sectional view of the parts shown in Fig. 1;

Fig. 3 is a view similar to Fig. 2, with plaster applied;

Fig. 4 is a view similar to Fig. 1 of a somewhat modified form of the invention;

Fig. 5 is a cross sectional view of the parts shown in Fig. 4;

Fig. 6 is a view similar to Fig. 5 with the plaster applied; and

Fig. 7 is an enlarged detail view of one of the plaster holding perforations or recesses.

1, indicates a main body portion of a fiber board known to the trade as "insulite." It is composed of large sliver like particles 2, often one sixteenth or one thirty second of an inch in width and say one half an inch long. These sliver like fibers give great porosity to the mass 1, but they render the binding together of the particles more difficult. To partly overcome this last named objection, while still retaining the greater heat insulating qualities due to the higher porosity, given by the slivers 2, said insulite has long hair like fibers 3 which serve to bind together said slivers 2. These fibers 3 are often one or two inches long, and are say one

one hundredth or one two hundredth of an inch in diameter. These said fibers 2 and 3 make an exceedingly porous mass, but it is loosely compacted, and has not a sufficient body to it. To remedy this defect, said insulite further is provided with short fine hair like fibers 4 which are say one two hundredth of an inch in diameter, or smaller still, and say about one fourth inch long, or even shorter. These said fibers 4 serve as a filler for the mass, and may be associated with a substantial percentage of other filler fibers, such as those usually employed in paper making. When the mass is constructed as above disclosed such a large quantity of air is entrained in the pores thereof that there results a board having not only an abnormal lightness and porosity but it possesses the valuable property of having abnormal heat insulating qualities, and therefore, it possesses many of the physical characteristics of cork. In fact, such a board will seldom be found to have a specific gravity exceeding (.4) four tenths, and it often will be found to have a specific gravity not exceeding (.2) two tenths. It is readily produced in thicknesses greater than those possessed by other fiber paper boards, and as the above mentioned fibers are truly felted together, during the manufacture of the board, said board does not readily peel or flake off in layers as do paper boards.

The physical properties, and especially the abnormal and extraordinarily high heat insulating qualities of this particular insulite board, render it peculiarly adapted for walls of inexpensive buildings when stucco, cement, or plaster is applied thereto, but its unusually porous nature permits it to more readily absorb moisture than other paper boards, especially where the fibers are torn to provide recesses, or holding perforations, for the plaster, stucco, or cement, as must be done. This objection is aggravated by reason of the fact that cement itself, as well as Portland cement-stucco, absorbs water readily. Therefore, for this reason alone, it is very desirable to render the insulite material waterproof, but again, it has been found that if the waterproofing material extends throughout the mass of the insulite, it has a decided objection in that it reduces somewhat its heat insulating properties.

Not only does the cement or stucco material readily absorb water, as above stated, but it, owing to its alkaline character, at

tacks the wood pulp constituents of the insulite, and this attacking action is enhanced by the moisture which has been absorbed by the cement material.

5 To avoid these last mentioned objections, instead of impregnating the insulite throughout its body with a waterproofing material, I coat only the outer surfaces of said insulite material, with a water resisting compound, 10 such as tar, asphalt, pitch or boiled linseed oil. This coating cannot be applied by the usual process of dipping, etc., because, the very porous nature of the insulite material would cause the waterproofing material to 15 readily soak throughout the mass, and thus reduce the heat insulating properties, as above mentioned, as well as waste the waterproofing material. Therefore, I spray the outer surfaces of the insulite material, with 20 any suitable water repelling material, such for example as a solution of asphalt and take care that the spray enters the perforations or recesses with which the body of the insulite is provided.

25 Accordingly, in carrying out this invention, I provide the body of insulite 1, above mentioned, I further cut, mold or otherwise produce in said body, suitable recesses such as 6, which are preferably undercut as 30 shown, and I thoroughly spray the said recesses as well as the entire outer surface of the board 1 with a suitable water proofing material 7, which material only penetrates a limited distance into the interior of the 35 board 1, and forms a protecting coating as shown. To the material thus coated, I next apply a suitable plastic such as ordinary plaster, cement, or stucco, 8 which fills said recesses 6 as shown, but which is nevertheless 40 less separated from the body of the insulite 1 by the waterproofing material 7, as shown. In the modified forms of the invention illustrated in Figs. 4, 5, and 6, the same process is carried out, but the recesses or indentations 45 9 are of a different form from the recesses 6, shown in the preceding figures, and further, they are pointed in different directions as indicated in dotted lines in said figures, for the purpose of giving a better hold 50 to the plaster material 8. It will now be clear that by providing the peculiar com-

position board known as insulite, and by protecting its outer surfaces thoroughly from moisture, I am enabled to produce a plaster board which is free from the objections above noted, and which yet possesses the very high heat insulating qualities in- 55 sultite is known to possess.

It is obvious that those skilled in the art may vary the details of the procedure as well 60 as the construction without departing from the spirit of the invention, and therefore, I do not wish to be limited to the above disclosure except as may be required by the 65 claims.

What I claim is:—

1. A plaster board composed of sliver like fibers to give porosity, long hair like fibers to act as a binder, and short fibers to act as a filler, said body portion being abnormally 70 light and porous and possessing abnormally high heat insulating qualities said body portion also provided with recesses in its surface and with a layer of plastic material entering said recesses; said body portion further provided between said plastic material and said fibers with a thin layer of water proofing material preferably sprayed onto said fibers, 75 substantially as described.

2. A plaster board composed of sliver like 80 fibers to give porosity, long hair like fibers to act as a binder, and short fibers to act as a filler, said body portion having a specific gravity less than .4 and possessing abnor- 85 mally high heat insulating qualities; said body portion also provided with recesses in its surface, and with a layer of plastic material having caustic properties entering said recesses; said body portion further provided between said plastic material and said fibers 90 to prevent the caustic action of said plastic material with a thin layer of water proofing material preferably sprayed onto and not substantially penetrating the mass of said fibers, substantially as described. 95

In testimony whereof I affix my signature, in presence of two witnesses.

TREADWAY B. MUNROE.

Witnesses:

H. STEADMAN,  
L. H. JEFFRES.